

July 5, 1966

A. A. POPOFF

3,258,841

METHOD FOR EXPLOSIVELY BONDING METAL LAYERS

Filed Jan. 23, 1963

3 Sheets-Sheet 1



Fig. 1.



Fig. 2.



Fig. 3.



Fig. 4.



Fig. 5.



Fig. 6.



Fig. 7.

INVENTOR  
ALEXIS A. POPOFF  
BY *John H. Tregoning*

July 5, 1966

A. A. POPOFF

3,258,841

METHOD FOR EXPLOSIVELY BONDING METAL LAYERS

Filed Jan. 23, 1963

2 Sheets-Sheet 2



Fig. 8.



Fig. 9.



Fig. 12.



Fig. 10.



Fig. 11.

INVENTOR

BY ALEXIS A. POPOFF

*John H. Tregoming*

1

3,258,841  
**METHOD FOR EXPLOSIVELY BONDING  
METAL LAYERS**

Alexis A. Popoff, Woodbury, N.J., assignor to E. I. du Pont de Nemours and Company, Wilmington, Del., a corporation of Delaware

Filed Jan. 23, 1963, Ser. No. 253,485  
6 Claims. (Cl. 29—486)

The present invention relates to an improved method of bonding metals by explosive means.

A process has been described recently for bonding metal layers to form a multilayered body by supporting a metal cladding layer a distance of at least 0.001 inch from a metal base layer, placing a layer of an explosive having a detonation velocity less than 120% of the sonic velocity of the metal having the highest sonic velocity in the system on the outside surface of the metal cladding layer, and initiating the explosive so that detonation is propagated parallel to the metal layers. Although the bonding obtained by this process is excellent, some areas around the edges of the composite systems may be left unbonded. This problem is particularly acute when the metal layers and the explosive layer are substantially rectangular and the explosive layer is initiated by means of a blasting cap, detonating cord, or some other device positioned at a point or points along one edge of the layer. In the majority of cases the largest unbonded zone extends over an essentially rectangular area along that edge of the composite system which was contiguous to the point or points of initiation.

This difficulty is overcome and a completely bonded clad metal system is produced by

(1) Providing metal extension pieces on at least one of the edges of a metal cladding layer, each of said metal extension pieces being contiguous to an edge of the metal cladding layer for substantially the length of said edge, extending in a direction perpendicular to said length of the edge of the cladding layer a distance at least four times the thickness of the metal cladding layer, and having an areal density of at least 50% and no more than 150% of the areal density of said metal cladding layer,

(2) Supporting said metal cladding layer substantially parallel to and separated by a distance of at least 0.01 inch from a metal base layer,

(3) Covering the area defined by the outside surfaces of said metal cladding layer and extension pieces with a layer of a detonating explosive having a detonation velocity between about 1200 meters per second and 120% of the sonic velocity of the metal having the highest sonic velocity in the system, and

(4) Initiating the explosive layer so that detonation is propagated parallel to the plane of the metal cladding layer and the metal extension pieces are sheared from the metal cladding layer.

For a more complete understanding of the process of the present invention reference is now made to the attached drawings in which like numbers indicate similar elements and in which

FIGURES 1-7 represent cross-sectional views of assemblies which may be used for the practice of the present invention, and

FIGURES 8-12 represent top views of portions of assemblies which may be used for the practice of the present invention.

In FIGURES 1-7 metal cladding layer 1 to which are attached metal extension pieces 2 is positioned above metal base layer 3 (supporting means are not shown). The upper surfaces of metal cladding layer 1 and metal extension pieces 2 are covered with a layer of a detonating explosive 4 to which is attached an electric blasting cap

2

5 having lead wires 6 to a source of electric current. In FIGURE 4 the joints between metal cladding layer 1 and metal extension pieces 2 are covered with metal strips 7 which serve as "gas blockers" preventing detonation gases from flowing through these joints and entering the space between metal layers 1 and 3.

FIGURES 8-12 depict the upper surfaces of the metal extension pieces 2 and of the metal cladding layer 1 to which the metal extension pieces 2 are attached. The term "metal cladding layer" in this application refers to that layer which is explosively bonded to the metal base layer by the process of the present invention. In FIGURES 8-12 the upper surface of each metal cladding layer 1 is defined by the area ABCD and the hatched areas represent the upper surfaces of the metal extension pieces 2. In FIGURES 8-11 the metal cladding layer 1 and the metal extension piece(s) 2 can comprise adjacent sections of a single metal plate the upper surface of which is defined, for example, in FIGURE 8, by the area ABEF. Alternatively, the metal extension piece(s) 2 can comprise, as for example, in FIGURE 7, a separate metal strip or bar the upper surface of which is defined by the area DCEF and which is attached to metal cladding layer 1 along the edge DC.

25 Alternatively, the metal extension pieces 2 can be provided in the form of a metal "picture frame" as shown in FIGURES 7 and 12. In FIGURE 12, the broken lines, AB, BC, CD, and DA, correspond to the edges of metal cladding layer 1 which are overlapped by the edges of the extension pieces 2. Obviously, metal extension pieces 2 can be attached to one, two, three, or four edges of metal cladding layer 1 and can comprise integral parts of a single metal plate or layer or separate pieces of metal attached to edges of metal cladding layer 1 by any of several methods which will be more fully described hereinafter.

30 The term "metal" in this application includes any elemental metal or mixture of elemental metals, e.g., an alloy. The metal layers are generally substantially rectangular and it is toward the production of substantially rectangular clad metal systems that this invention is directed.

35 The composition, loading, and confinement of the explosive layer, and the particular device(s) used to initiate the explosive layer must be selected so that the detonation velocity of the explosive remains within the limits given above and so that detonation is propagated parallel to the metal cladding layer.

40 The minimum separation or standoff between the metal layers which results in a strong, continuous metal-to-metal bond is about 0.01 inch. The optimum size of this standoff depends upon a number of factors including the metal cladding layer thickness and density and the explosive loading, confinement, and detonation velocity. The specific spacing members used to provide this standoff must not be such as to introduce a large mass of foreign material or cause entrapment of air in the bond zone between the metal layers.

45 Although there is no intention to be limited by any theory of operation it is believed that unbonded zones around the edges of an explosively clad metal system are attributable, at least in part, to a lag in the velocity of the edges of the metal cladding layer as compared with the velocity of the center of the layer when the metal cladding layer is propelled by the pressure exerted by a uniform layer of explosive. This lag in velocity is caused by the boundary conditions which exist along the free surfaces, i.e., at the edges of the explosive layer. Since the free surfaces must remain at atmospheric pressure, when the explosive is initiated, rarefaction waves are formed at the edges of the explosive layer. Lower pressure is

exerted on the edges of the metal cladding layer than is exerted on the center of the layer and lower velocity is imparted to the edges than is imparted to the center of the layer. Thus, each edge strikes the corresponding edge of the base layer with insufficient velocity to produce the plastic deformation required to establish a bond.

When the explosive is initiated at a point or points along one edge of the layer, the problem of unbonded zones is particularly acute along that edge of the clad metal system which corresponds to the "initiation edge" of the layer of explosive. Although the cause of this unique difficulty is not fully understood, it is probable that a number of factors are involved.

Explosive bonding within the sense and scope of this invention generally is accompanied by a "jetting" phenomenon. When the metal cladding and base layers collide at an angle which is critical for a given value of the sonic velocity of the metal layers and the detonation velocity of the explosive layer, a jet composed of molten surface portions of both metal layers is formed, circulated, and solidified between the layers. However, when the explosive is initiated at a point or points along one edge of the layer, for a very small distance, this edge of the metal cladding layer may be propelled essentially normal to the metal base layer and thus fail to form the critical angle necessary for jetting. The effects of this geometrical consideration, the edge lag described above, and the anomalies associated with start-up of detonation of the explosive layer combine to intensify the problem of unbonded zones along the initiation edge. When the explosive is initiated at one corner of the layer this combination of factors is detrimental to bonding along the two edges adjacent to the initiation corner and when one entire edge of the layer is initiated simultaneously, for example, by means of a line wave generator the geometry and dynamics of the system often lead to large unbonded zones along all of the edges except that edge directly opposite to the initiation edge. Furthermore, even in cases in which "jetting" occurs over the entire interface between the metal layers detonation gases often enter the space between the two layers and prevent formation of a good metal-to-metal bond around the periphery of the system.

The average width of the unbonded zones along the edges of the cladding layer increases with the thickness of the cladding layer. For example, when the cladding layer is  $\frac{1}{16}$  inch thick unbonded zones at least  $\frac{1}{4}$  inch wide are observed and when the cladding layer is more than  $\frac{1}{16}$  inch thick there is at least a proportional increase in the width of the unbonded zones, i.e., the width of the unbonded zones generally is at least about 4 times the thickness of the cladding layer. However, if extension pieces  $\frac{1}{16}$  inch thick and  $\frac{1}{4}$  inch wide ( $\frac{1}{4}$  inch wide not counting the overlap when using extension pieces as shown in FIGURE 12) are attached to one or more of the edges of the  $\frac{1}{16}$ -inch thick cladding layer, i.e., so that each extension piece extends  $\frac{1}{4}$  inch normal to the length of the edge to which it is attached, the lagging edges and their attendant difficulties are effectively removed from the area to be bonded. The width of a metal extension piece normal to the edge to which it is attached, e.g., the width DF or CE in FIGURE 7 or 12, must be at least 4 times the thickness of the metal cladding layer in order to insure complete bonding along the edge to which it is attached, i.e., the edge DC in FIGURE 7. When the cladding layer is very thin, for example, on the order of a few mils thick, the extension pieces are generally considerably wider than four times the thickness of the cladding layer simply because of the difficulty of working with narrow strips of thin metal sheets. However for obvious economic reasons, the width of the extension pieces should be kept as close to the minimum as possible.

The number of extension pieces which must be used to insure an essentially completely bonded clad metal system depends, among other things, upon the thickness and shape of the cladding layer and upon the location of

the point(s) of initiation of the explosive layer. When the cladding layer is relatively thin the unbonded zones attributed simply to edge lag are relatively narrow and the cost of trimming the unbonded edges may be comparable to or less than the cost of providing extension pieces on all four edges of the cladding layer. However, in such cases, as explained above the unbonded zones along the edge or edges of the clad metal system which are contiguous to the point or points of initiation of the layer of explosive are considerably wider than those along the other edges of the system. Thus, referring to FIGURE 7, for example, if the layer of explosive is to be initiated at a point along that edge of the layer which corresponds to edge DC of the metal cladding layer a single metal extension piece attached as shown in FIGURE 7 is sufficient to eliminate unbonded zones of any significant width. Obviously the layer of explosive covers the surface of the extension piece as well as that of the metal cladding layer and is initiated at a point along the line FE. Other practical arrangements for cladding with a relatively thin metal cladding layer include those illustrated in FIGURES 9 and 10. In the former case the explosive is initiated at that corner of the layer of explosive which is contiguous to the juncture between the extension pieces, as in Example 5. The arrangement shown in FIGURE 10 can be used in conjunction with a linewave generator which initiates the explosive along the edge opposite to that edge of the cladding layer to which no extension piece is attached as in Example 7. When the cladding layer is relatively thick, four extension pieces are generally necessary to insure a completely bonded clad metal system. As mentioned above, each extension piece is at least four times as wide as the thickness of the cladding layer. When the explosive is initiated at a point or points along one edge of the explosive layer it is desirable to use a metal extension piece of more than the minimum width along the contiguous edge of the cladding layer. This provides additional protection to counteract the problems associated with the initiation edge. If center initiation is used this precaution is unnecessary.

Ideally the layer of explosive detonates parallel to the plane of the metal cladding layer and accelerates the extension pieces and the cladding layer with essentially uniform velocity. When the joint between an extension piece and an edge of the metal cladding layer is continuous and the areal densities of the extension piece and cladding layer are comparable, e.g., as shown in FIGURE 1, there is essentially no velocity differential across the joint. However, we have found that the areal density of an extension piece can vary between about 50 and 150 percent of the areal density of the cladding layer and still be effective in essentially eliminating unbonded zones along the edge to which it is attached. When the areal density of the extension piece is outside these limits the velocity differential between the extension piece and the cladding layer which is due to the edge-lag effect described above is insignificant compared to the velocity differential across the joint which is due to the widely differing areal densities of the extension piece and cladding layer. If the areal density of the extension piece is less than 50 percent of that of the cladding layer the extension piece is accelerated to a higher velocity than is the cladding layer and the joint between the extension piece and the cladding layer is put under such strain that it often breaks before the bond between the edges of the cladding and base layers is established thus permitting, for example, entry of detonation gases into the space between the layers and preventing formation of a good metallurgical bond between the two layers. If the areal density of the extension piece is more than 150 percent of that of the cladding layer, the cladding layer is accelerated to a higher velocity than is the extension piece and again the joint between the cladding layer and extension piece is strained with the deleterious effects described above.

Obviously, the strength of this joint will vary depending upon, for example, whether the cladding layer and extension piece are sections of a single plate or separate pieces of metal joined by welding, epoxy resin, etc. Often it is sufficient to simply lay the "picture frame" shown in FIGURE 12 on top of the cladding layer. Detonation of the explosive layer effectively shears and removes the extended portions of the "picture frame" from the clad metal system and the overlapped portions of the "picture frame" either are shattered and blasted away from the system during detonation or are easily removed after detonation.

For most systems the above-defined limits with respect to areal density represent practical limits within which the process of the present invention can satisfactorily be carried out. These limits can be satisfied in a number of ways. First, the extension pieces can be of the same thickness and composition as the metal cladding layer. One convenient method of practicing the present invention comprises using a metal cladding layer which is oversize with respect to the base layer on one or more edges as described above in connection with FIGURE 7 and described hereinafter in Examples 1, 3 and 6. If, however, the cladding layer is so thick that the extending edges are not sheared during the explosive process, the extension pieces can be prepared from metal plates of the same thickness and composition as the cladding layer and can be attached to the cladding layer by a bond which does break or "give" during the cladding process.

Since the cladding layer often comprises an expensive metal which is bonded to the base layer to give the composite some specific desirable property such as high corrosion resistance, the cost of extension pieces of the same metal as the cladding layer is often prohibitive. In such cases the extension pieces can be of the same thickness as the cladding layer but made of a different metal having a density comparable to that of the cladding layer as in FIGURE 1.

Extension pieces of substantially higher or lower density (weight per unit volume) than the cladding layer are also satisfactory. In order to compensate for the difference in density the thickness of the extension pieces is adjusted so that the weights per unit area or areal densities of the extension pieces and the cladding layer are within the limits defined above. FIGURES 2, 5, and 6 illustrate assemblies wherein the extension pieces are thicker than the cladding layers. The inner corners of the extension pieces can be square as in FIGURES 2 and 5 or obtuse angles as in FIGURE 6. FIGURE 3 illustrates an assembly in which the extension pieces are thinner than the cladding layer.

The joints between the cladding layer and the extension pieces must be strong enough to support the weight of the explosive layer and any confining medium which is used and weak enough to allow the extension pieces to be completely sheared from the cladding layer during the explosive operation. If the bonds between the cladding layer and extension pieces are too strong or if obstructions which offer sufficient resistance to the motion of the extension pieces are placed below the extension pieces, the extension pieces spring back or spall or partially shear and pull the cladding and base layers apart thus preventing bonding and/or allowing entry of detonation gases into the space between the two layers. Suitable methods of attachment are, for example, cement, epoxy resin, and shallow, metallic welds.

If the edges of the cladding layer are rough or uneven it is difficult to provide extension pieces flush with the edges of the layer. In such cases it is advisable to fill the gaps with a material such as a metal-filled epoxy resin or solder which serves as a method of attaching the extension pieces to the cladding layer and has a density in the range of that of the metal extension pieces and cladding layer. The entry of detonation gases into the space between the metal layers is seriously detrimental

to the formation of a good bond. The detonation gases can, for example "cushion" and thus reduce the velocity of the cladding layer and/or react with the metal of the cladding or base layer to form a deleterious oxide phase.

5 Filling the gaps between the edges of the cladding layer and extension pieces can prevent the detonation gases from flowing through the joints and between the metal layers. However, use of metal strips as "gas blockers" arranged over the joints as in FIGURE 4 or of the assembly shown in FIGURES 7 and 12 is a necessary precaution in many cases.

The configuration of the joints between the extension pieces and the cladding layer is not critical provided that the extension pieces shear from the cladding layer and detonation gases are prevented from entering the bonding zone. A simple butt joint as illustrated in FIGURES 1 to 6 is a particularly convenient configuration. However any practicable beveled or notched joint is satisfactory. The extension pieces can be rectangular as illustrated in FIGURES 8 to 11 or trapezoidal as illustrated in FIGURE 12 in which case a joint between any two extension pieces will form obtuse angles with the joints between the extension pieces and the corresponding edges of the cladding layer.

15 20 25 The following examples illustrate some of the modifications of the process of the present invention. They are intended as illustrative only, however, and are not to be considered as exhaustive or limiting.

#### Example 1

30 A stainless steel plate  $\frac{1}{16}$  inch thick, 6 inches wide, and 10 inches long is positioned above and parallel to a mild steel plate  $\frac{1}{2}$  inch thick, 6 inches wide, and 9 inches long so that a 1-inch segment of the length of the stainless steel plate extends beyond the mild steel plate substantially as illustrated in FIGURE 1. The adjacent surfaces of the two plates are separated by a distance of .060 inch maintained by shim steel cups .060 inch deep and  $\frac{1}{8}$  inch in diameter, one of which is spot welded in each of the four corners of the upper surface of the mild steel plate. The upper surface of the stainless steel plate is covered with a sheet of a fibrous explosive composition comprising 75 parts pentaerythritol tetranitrate, 17.5 parts of a butadiene-acrylonitrile rubber, and 7.5 parts paper pulp and having a weight distribution of 4 grams per square inch. This explosive detonates at a velocity of about 3600 meters per second. An electric blasting cap having lead wires to a source of electric current is attached to the center of that edge of the layer of explosive which is contiguous to the extended edge of the stainless steel plate. The entire assembly is covered with a pile of sand 1 foot deep. A piece of cardboard glued to the extended edge of the stainless steel plate perpendicular to the plate keeps the space directly beneath the stainless steel extension free of sand. The blasting cap which is actuated by application of electric current initiates the layer of explosive. During detonation, the stainless steel extension is sheared from the plate and a stainless steel-on-mild steel composite 6 inches wide and 9 inches long is formed. Ultrasonic probing reveals no unbonded zones around the edges of the metallurgically bonded clad metal system.

#### Example 2

65 70 75 A clad metal system of the composition, dimensions, and quality described in Example 1 is prepared using the materials and a modification of the technique described in Example 1. In this example the stainless steel plate is  $\frac{1}{16}$  inch thick, 6 inches wide, and 9 inches long. A piece of mild steel  $\frac{1}{16}$  inch thick, 1 inch wide and 6 inches long is butted along its length against one of the 6-inch edges of the stainless steel plate and glued in place with epoxy resin thus forming a mild steel extension to the stainless steel plate substantially as illustrated in FIGURE 1. During detonation, the mild steel extension is sheared from the stainless steel plate and a stainless steel-on-mild steel composite 6 inches wide and 9 inches long

is formed. Again, ultrasonic probing reveals no unbonded zones around the edges of the metallurgically bonded composite.

*Example 3*

A stainless steel plate  $\frac{1}{8}$  inch thick, 7 inches wide and  $10\frac{1}{2}$  inches long is positioned above and parallel to a mild steel plate  $\frac{1}{2}$  inch thick, 6 inches wide and 9 inches long so that one of the 7-inch edges of the stainless steel plate extends 1 inch beyond the adjacent 6-inch edge of the mild steel plate and each of the other 3 edges of the stainless steel plate extends  $\frac{1}{2}$  inch beyond the corresponding adjacent edge of the mild steel plate. The adjacent surfaces of the two plates are separated by a distance of .060 inch maintained as in Example 1. The upper surface of the stainless steel plate is covered with a layer of a grained amatol explosive comprising 50 parts ammonium nitrate and 50 parts trinitrotoluene. The layer of explosive, which is contained by a rectangular wooden frame about  $\frac{1}{8}$  inch thick and 1 inch high placed on the perimeter of the upper surface of the stainless steel plate, is  $\frac{3}{4}$  inch thick and has a detonation velocity of about 3500 meters per second. An electric blasting cap is attached to the wooden frame in the center of that edge of the layer of explosive which is contiguous to the edge of the stainless steel plate which extends 1 inch beyond the mild steel plate. The layer of explosive is covered with a sheet of waxed paper and the entire assembly is covered with a pile of sand 5 feet deep. Pieces of cardboard glued around the edges of the stainless steel plate perpendicular to the plate keep the space directly beneath the extensions free of sand. The blasting cap is actuated by application of electric current and initiates the layer of explosive. During detonation the stainless steel extensions are sheared from the plate and a stainless steel-on-mild steel composite 6 inches wide and 9 inches long is formed. Ultrasonic probing reveals no unbonded zones around the edges of the metallurgically bonded clad metal system.

*Example 4*

A clad metal system of the composition, dimensions and quality described in Example 3 is prepared using the materials and a modification of the technique described in Example 3. In this example the stainless steel plate is  $\frac{1}{8}$  inch thick, 6 inches wide, and 9 inches long. A piece of mild steel  $\frac{1}{8}$  inch thick, 1 inch wide, and  $6\frac{1}{2}$  inches long is butted along its length against one of the 6-inch edges of the stainless steel plate so that a  $\frac{1}{2}$ -inch segment of the length of the mild steel extends beyond the end of the 6-inch edge of the stainless steel plate. A second piece of mild steel  $\frac{1}{8}$  inch thick,  $\frac{1}{2}$  inch wide and  $9\frac{1}{2}$  inches long is butted along its length against one of the 9-inch edges of the stainless steel plate so that one of the ends is flush with the  $90^\circ$  angle formed by the extension of the first piece of mild steel and the 9-inch edge of the stainless steel plate and the other end extends  $\frac{1}{2}$  inch beyond the 9-inch edge of the stainless steel plate. A third piece of mild steel  $\frac{1}{8}$  inch thick,  $\frac{1}{2}$  inch wide, and  $6\frac{1}{2}$  inches long is butted along its length against the second 6-inch edge of the stainless steel plate so that one of the ends is flush with the  $90^\circ$  angle formed by the extension of the second piece of mild steel and the second 6-inch edge of the stainless steel plate and the other end extends  $\frac{1}{2}$  inch beyond the second 6-inch edge of the stainless steel plate. A fourth piece of mild steel  $\frac{1}{8}$  inch thick,  $\frac{1}{2}$  inch wide and 10 inches long is butted along its length against the remaining 9-inch edge of the stainless steel plate so that one of the ends is flush with the  $90^\circ$  angle formed by the third piece of mild steel and the 9-inch edge of the stainless steel plate and the other end extends 1 inch beyond the end of the 9-inch edge of the stainless steel plate and is flush with the 1-inch edge of the first piece of mild steel. The four pieces of mild steel are glued in place with epoxy resin thus forming a 1-inch extension on one end of the stainless steel plate

and  $\frac{1}{2}$  inch extensions on the remaining 3 sides of the plate substantially as illustrated in FIGURE 9.

The cladding process is carried out as in Example 3. During detonation all four mild steel extensions are sheared from the stainless steel plate and a stainless steel-on-mild steel composite 6 inches wide and 9 inches long is formed. Ultrasonic probing reveals no unbonded zones around the edges of the metallurgically bonded clad metal system.

10

15

20

25

30

35

40

45

50

55

60

65

70

75

*Example 5*

A nickel plate  $\frac{1}{8}$  inch thick, 18 inches wide, and 18 inches long is positioned above and parallel to a mild steel plate  $\frac{1}{2}$  inch thick, 18 inches wide and 18 inches long. The adjacent surfaces of the two plates are separated by a distance of .060 inch maintained as in Example 1. A piece of mild steel  $\frac{1}{8}$  inch thick, 1 inch wide and 18 inches long is butted along its length against one of the 18-inch edges of the nickel plate. A second piece of mild steel  $\frac{1}{8}$  inch thick, 1 inch wide and 19 inches long is butted along its length against an adjacent 18-inch edge of the nickel plate so that one end extends 1 inch beyond the end of the 18-inch edge of the nickel plate and is flush with the 1 inch edge of the first piece of mild steel. The two pieces of mild steel are glued in place with epoxy resin thus forming 1-inch extensions on 2 adjacent edges of the nickel plate. The upper surfaces of the nickel plate and the mild steel extensions are covered with a  $\frac{3}{4}$ -inch layer of the explosive described in Example 3, contained in a wooden frame as in Example 3. An electric blasting cap is attached to the wooden frame in that corner of the layer of explosive which is contiguous to the corner at which the mild steel extension pieces meet. The layer of explosive is covered with a sheet of waxed paper and the entire assembly is covered with a pile of sand 5 feet deep. Pieces of cardboard glued to the edges of the mild steel extension pieces as in the preceding examples keep the space directly beneath the extension pieces free of sand. The blasting cap is actuated by application of electric current and initiates the layer of explosive. During detonation the two mild steel extension pieces are sheared from the nickel plate and a nickel-on-mild steel composite 18 inches wide and 18 inches long is formed. Ultrasonic probing reveals no unbonded zones along the edges of the metallurgically bonded clad metal system.

*Example 6*

A copper plate  $\frac{1}{8}$  inch thick, 7 inches wide, and 13 inches long is positioned above and parallel to a mild steel plate  $\frac{1}{2}$  inch thick, 6 inches wide, and 12 inches long so that one of the 7-inch edges of the copper plate extends 1 inch beyond the adjacent 6-inch edge of the mild steel plate and each of the 13-inch edges of the copper plate extends  $\frac{1}{2}$  inch beyond the corresponding, adjacent 12-inch edge of the mild steel plate. The adjacent surfaces of the two plates are separated by a distance of .060 inch maintained as in Example 1. The upper surface of the copper plate is covered with a  $\frac{3}{4}$ -inch layer of the explosive described in Example 3, contained in a wooden frame as in Example 3. An electric blasting cap is attached to the wooden frame in the center of that edge of the layer of explosive which is contiguous to the edge of the copper plate which extends 1 inch beyond the mild steel plate. The layer of explosive is covered with a sheet of waxed paper and the entire assembly is covered with a pile of sand 5 feet deep. Pieces of cardboard glued to the three extended edges of the copper plate as in the preceding examples keep the space directly beneath the extensions free of sand. The blasting cap is actuated by application of electric current and initiates the layer of explosive. During detonation the copper extensions are sheared from the plate and a copper-on-mild steel composite 6 inches wide and 12 inches long is formed. Ul-

trasonic probing reveals no unbonded zones along the edges of the metallurgically bonded clad metal system.

*Example 7*

A clad metal system of the composition, dimensions and quality described in Example 6 is prepared using the materials and a modification of the technique described in Example 6. In this example the copper plate is  $\frac{1}{8}$  inch thick, 6 inches wide, and 12 inches long. A piece of mild steel  $\frac{1}{8}$  inch thick, 1 inch wide and  $6\frac{1}{2}$  inches long is butted along its length against one of the 6-inch edges of the copper plate so that a  $\frac{1}{2}$ -inch segment of the length of the mild steel extends beyond the end of the 6-inch edge of the copper plate. A second piece of mild steel  $\frac{1}{8}$  inch thick,  $\frac{1}{2}$  inch wide, and 12 inches long is butted along its length against one of the 12-inch edges of the copper plate so that one of the ends is flush with the  $90^\circ$  angle formed by the extension of the first piece of mild steel and the 12-inch edge of the copper plate. A third piece of mild steel  $\frac{1}{8}$  inch thick,  $\frac{1}{2}$  inch wide, and 13 inches long is butted along its length against the second 12-inch edge of the copper plate so that one end extends 1 inch beyond the end of the 12-inch edge of the copper plate and is flush with the 1-inch edge of the first piece of mild steel. The three pieces of mild steel are glued in place with epoxy resin thus forming a 1-inch extension on one end of the copper plate and  $\frac{1}{2}$ -inch extensions on the two long edges of the copper plate.

The cladding process is carried out substantially as in Example 3. However, in this example the layer of explosive is initiated by a triangular line-wave generator which is attached along that edge of the layer of explosive which is contiguous to the edge of the 1-inch mild steel extension. The line-wave generator is initiated by an electric blasting cap attached to the apex of the generator. During detonation the three mild steel extensions are sheared from the copper plate and a copper-on-mild steel composite 6 inches wide and 9 inches long is formed. Ultrasonic testing reveals no unbonded zones along the edges of the metallurgically bonded clad metal system.

*Example 8*

A tantalum plate .040 inch thick, 12 inches wide and 24 inches long is positioned above and parallel to a mild steel plate  $\frac{3}{8}$  inch thick, 12 inches wide, and 24 inches long. The adjacent surfaces of the two plates are separated by a distance of .045 inch maintained by two shim steel ribbons one of which is spot welded along the length of the upper surface of the mild steel plate, parallel to and 1 inch in from each of the 24-inch edges of the plate. Each of these ribbons is .001 inch thick and .045 inch wide, and is deformed normal to its thickness into a sine wave configuration of 3 cycles per linear inch and approximately .050 inch amplitude. Each ribbon is placed "on edge" on the surface of the plate, i.e., so that the .045-inch dimension of the ribbon is perpendicular to the plane of the plate. Four mild steel extension pieces are attached to the tantalum plate as described in Example 4. However, in this case each of the pieces of mild steel is .060 inch thick and 1 inch wide. The mild steel extension pieces attached to the 12-inch edges of the tantalum plate are 13 inches long and those attached to the 24-inch edges of the plate are 25 inches long. The pieces of mild steel are glued in place with epoxy resin thus forming 1-inch extensions on each of the four edges of the tantalum plate substantially as illustrated in cross-section in FIGURE 2. The upper surfaces of the tantalum plate and the mild steel extension pieces are covered with a layer of a grained soda amatol explosive comprising equal parts of ammonium nitrate, sodium nitrate, and trinitrotoluene. The layer of explosive which is contained in a wooden frame as in Example 3 is .375 inch thick over the mild steel extension pieces and .395 inch thick over

the tantalum plate. The average weight distribution of the explosive is approximately 6 grams per square inch and the detonation velocity is 3100 meters per second. An electric blasting cap is attached to the wooden frame in the center of one of the edges of the layer of explosive which is contiguous to one of the 13-inch extension pieces and the layer of explosive is covered with a sheet of waxed paper. The entire assembly is covered with a wooden box which is in turn covered with a pile of sand. The blasting cap is actuated by application of electric current and initiates the layer of explosive. During detonation, the four mild steel extension pieces are sheared from the tantalum plate and a tantalum-on-mild steel composite 12 inches wide and 24 inches long is formed. Ultrasonic probing reveals no unbonded zones along the edges of the metallurgically bonded clad metal system.

*Example 9*

A tantalum-on-mild steel composite of the dimensions described in Example 8 is prepared using the materials and a modification of the technique described in Example 8. However in this example each of the mild steel extension pieces is  $1\frac{1}{2}$  inches, rather than 1 inch wide, the two shorter pieces are  $12\frac{1}{2}$  inches long, and the two longer pieces are  $24\frac{1}{2}$  inches long. The four pieces are welded together to form a rectangular "picture frame," the perimeter of which is 14 inches wide by 26 inches long and each side of which is  $1\frac{1}{2}$  inches wide. The rectangular frame is laid on top of the cladding layer substantially as illustrated in FIGURE 12 so that a  $\frac{1}{2}$ -inch segment of each side of the frame overlaps the cladding layer. The frame is spot-welded in place and detonation is carried out substantially as in Example 8. However, in this example the blasting cap is positioned in the center of the layer of explosive. During detonation the portions of the frame which extend beyond the cladding layer are sheared from the assembly and the overlapping portions of the frame are effectively blasted free of the surface of the composite system. Ultrasonic probing reveals no unbonded zones along the edges of the metallurgically bonded clad metal system.

The invention having been fully described in the foregoing it is to be limited only by the following claims.

What is claimed is:

1. A process for producing a completely bonded clad metal system which comprises

(1) providing metal extension pieces on at least one of the edges of a substantially rectangular metal cladding layer, each of said metal extension pieces being contiguous to an edge of the metal cladding layer for substantially the length of said edge, extending in a direction perpendicular to said length of the edge of the cladding layer a distance of at least four times the thickness of the metal cladding layer, and having a weight distribution per unit area of at least 50% and no more than 150% of the weight distribution per unit area of the metal cladding layer,

(2) supporting said metal cladding layer substantially parallel to and separated by a distance of at least 0.01 inch from a substantially rectangular metal base layer,

(3) covering the area defined by the outside surfaces of said metal cladding layer and extension pieces with a layer of a detonating explosive having a detonation velocity between about 1200 meters per second and 120% of the sonic velocity of the metal having the highest sonic velocity in the system and

(4) initiating the explosive layer so that detonation is propagated parallel to the plane of the metal cladding layer and the metal extension pieces are sheared from the metal cladding layer.

2. A process as in claim 1 wherein a single metal extension piece is provided on one of the edges of the metal cladding layer and the explosive is initiated along that edge of the explosive layer which is parallel and adjacent

to that edge of the metal cladding layer to which the extension piece is attached.

3. A process as in claim 1 wherein one metal extension piece is provided on each of the four edges of the metal cladding layer.

4. A process as in claim 3 wherein the explosive is initiated substantially in the center of the layer of explosive.

5. A process as in claim 1 wherein metal extension pieces are provided on each of the two adjacent edges of the metal cladding layer and the explosive is initiated at that corner of the layer of explosive which is contiguous to the juncture between the metal extension pieces.

6. A process as in claim 1 wherein metal extension pieces are provided on three edges of the metal cladding layer and the explosive is initiated along that edge of the layer of explosive which is opposite to that edge of the metal cladding layer to which no extension piece is attached.

**References Cited by the Examiner**

**UNITED STATES PATENTS**

10 3,137,937 6/1964 Cowan et al. \_\_\_\_ 29—497.5 XR  
5 3,197,855 8/1965 Carter et al. \_\_\_\_\_ 29—470.1

JOHN F. CAMPBELL, *Primary Examiner*.